

# UNITED STATES PATENT OFFICE.

ALBERT W. SMITH AND WILLIAM R. VEAZEY, OF CLEVELAND, OHIO, ASSIGNEES TO THE DOW CHEMICAL COMPANY, OF MIDLAND, MICHIGAN, A CORPORATION OF MICHIGAN.

## METHOD OF MAKING METALLIC SODIUM.

1,334,179.

Specification of Letters Patent. Patented Mar. 16, 1920.

No Drawing.

Application filed October 12, 1918. Serial No. 257,895.

*To all whom it may concern:*

Be it known that we, ALBERT W. SMITH and WILLIAM R. VEAZEY, citizens of the United States, and residents of Cleveland, 5 county of Cuyahoga, and State of Ohio, have jointly invented a new and useful Improvement in Methods of Making Metallic Sodium, of which the following is a specification, the principle of the invention being 10 herein explained and the best mode in which we have contemplated applying that principle, so as to distinguish it from other inventions.

The method principally used in the electrolytic manufacture of metallic sodium, *i.e.*, the so-called Castner process, uses, as is well known, caustic soda (NaOH) as the material to be electrolyzed. A number of objections, however, are involved in the electrolysis of such material, one being the fact that only one-half of the electric current used is employed in producing sodium, the other half producing hydrogen by the electrolysis of the hydroxyl resulting from the 15 first step. Furthermore, the hydrogen and oxygen that are produced form an explosive mixture, with the result that the cells, when in operation, are continually subject to more or less dangerous explosions, which 20 at least serve to scatter fine particles of caustic in the atmosphere, if no more serious damage results; while the metallic sodium is soluble in fused sodium hydroxid, except 25 for a relatively limited temperature range, 30 so that it is necessary to confine the temperature within the cell to such prescribed 35 limits.

By reason of the aforementioned difficulties, and for the further reason that 40 some cheaper material than caustic would of course be desirable, a number of other compounds of sodium have heretofore been tried, but none successfully, so far as we are advised. Common salt (NaCl), which 45 would probably afford the cheapest source, unfortunately has so high a melting point that the sodium volatilizes and burns as it is formed, and the same is true of all the other available compounds or salts of sodium when used alone. It has also been attempted to work with mixtures of different salts. For example, caustic soda has been added to sodium carbonate ( $Na_2CO_3$ ), which latter alone fuses at too high a temperature, 50 in an endeavor to obtain a lower fusing 55

mixture; the result, however, is unsatisfactory because the caustic soda electrolyzes preferentially, and no advantage is accordingly gained.

The object of the present invention is to 60 provide a suitable mixture of sodium compounds or salts for use in this electrolytic process, whereby metallic sodium may be produced at a much lower cost, not only by reason of the cheapening of the source-material, but also by requiring less current and 65 otherwise simplifying and rendering less dangerous the operation itself. To the accomplishment of the foregoing and related ends, the invention, then, consists of the 70 steps hereinafter fully described and particularly pointed out in the claims.

The following description sets forth in detail one approved mode of carrying out the invention, such disclosed mode, however, constituting but one of the various 75 ways in which the principle of the invention may be used.

We have discovered that sodium compounds, and specifically sodium carbonate, 80 upon being added to sodium salts other than caustic soda, in proper proportions, will give a mixture capable of fusion at a low enough temperature to avoid the vaporization and burning of the metallic sodium. 85 At the same time, by a proper selection of these other sodium compounds, the carbonate or selected compound will electrolyze preferentially, which means that it is dissociated into its constituent elements at a 90 lower voltage than the admixed compounds.

As an example of a mixture of the sort generally referred to above, which has been found entirely satisfactory in actual practice, we take a mixture of sodium chlorid 95 with sodium carbonate, containing approximately two parts of the latter and one part of the former, for example, 35.6 parts of sodium chlorid and 64.4 parts of sodium carbonate by weight. This mixture is found 100 to have a melting point of approximately 600° C., and, upon being electrolyzed, produces metallic sodium of equal quality than that produced by the present commercial process. It will be obvious that by employing 105 this mixture we obviate entirely the use of caustic soda even as a component of the mixture, and thus not only eliminate what is a difficult material to handle, but also utilize the full effect of the electric current in 110

producing the desired product, *i. e.*, metallic sodium, instead of only fifty per cent. of such current.

Any suitable electrolytic cell may be employed in connection with the foregoing, a regular Castner caustic soda cell having been found entirely satisfactory in actual practice. With a mixture such as described above, it has been found possible to work with a potential of six volts between the terminals of the electric machine, indicating that only a few volts are required to effect dissociation.

Other modes of applying the principle of our invention may be employed instead of the one explained, change being made as regards the method herein disclosed, provided the step or steps stated by any of the following claims or the equivalent of such stated step or steps be employed.

We therefore particularly point out and distinctly claim as our invention:—

1. The method of making metallic sodium, which consists in electrolyzing sodium carbonate in a fused mixture of such salt and sodium chlorid, the ingredients being

so proportioned that such mixture has a lower melting point than either of its constituents.

2. The method of making metallic sodium, which consists in electrolyzing sodium carbonate in a fused mixture of such salt and sodium chlorid, the ingredients being so proportioned that such mixture has a melting point of approximately 600° C. 35

3. The method of making metallic sodium, which consists in electrolyzing sodium carbonate in a fused mixture of approximately two parts of such salt and one part of sodium chlorid, such mixture having a 40 lower melting point than either of its constituents.

4. The method of making metallic sodium, which consists in electrolyzing sodium carbonate in a fused mixture of 64.4 parts 45 of such salt and 35.6 parts of sodium chlorid, such mixture having a melting point of approximately 600° C.

Signed by us this 3rd day of October, 1918.

ALBERT W. SMITH.  
WILLIAM R. VEAZEY.